

# United States Patent Office

2,737,492

Patented Mar. 6, 1956

1

2,737,492

## LUBRICATING OIL COMPOSITIONS

Lindley Clair Beegle, Stamford, Charles E. Funk, Jr., Cos Cob, and Edwin Oscar Hook, New Canaan, Conn., assignors to American Cyanamid Company, New York, N. Y., a corporation of Maine

No Drawing. Application March 26, 1952,  
Serial No. 278,758

11 Claims. (Cl. 252—32.7)

The present invention relates to lubricating oil compositions, to lubricating oil additives to be incorporated therein, and includes methods of incorporating these additives in the lubricating oils and methods of producing such additives. More particularly, these lubricating oil compositions are those of the type known as crankcase oils for internal combustion engines and including heavy-duty oils for truck, bus, airplane and marine gasoline and diesel engines. More specifically, the present invention is concerned with improving agents or chemical additives for lubricating oils to increase the effective service life of engines using such oils under all types of operating conditions.

These additives are oil soluble and are effective to reduce or retard the oxidation or deterioration of the lubricating oil and to inhibit or mitigate the normal corrosive action of such oils or the decomposition products thereof on metallic parts. Additionally, these additives act as dispersants or anti-sludge agents to prevent the formation of hard sludge deposits due to sludge formation in the oil particularly at elevated temperatures to thereby maintain engine cleanliness. Although these compositions have particular applicability to mineral lubricating oils such as crankcase oils, it is to be appreciated that they find use in other oils such as animal and vegetable oils, including cutting oils, slushing oils, turbine oils, transformer oils, and the like oils, having tendencies to undergo oxidative changes.

When oils, such as conventional lubricating oils, are subjected to extended periods of use, especially at high operating temperatures, as in heavy duty service, they tend to decompose and for complex and objectionable oxidation and decomposition products including peroxides and organic acids. These substances possess corrosive and other deleterious properties and, unless neutralized or counteracted, will attack and damage engine metallic parts such as, for example, the hard bearing alloy metals as copper-lead and cadmium-silver. These acids, furthermore, may go through a chemical process whereby the molecules combine or polymerize into large aggregates to form lacquer-like deposits on or between the moving parts of the engine, causing excessive wearing or even sticking of operating parts. Even larger quantities of polymerization products remain dispersed in the partially oxidized oil and are readily precipitated to form a mayonnaise-like sludge when the engine cools or when fresh oil is added to the engine. These precipitated sludges become caked on the heated metal surfaces and reduce the effective life of the engine by preventing proper functioning of the parts thereof, such as by gumming up the piston rings to prevent proper piston action, or by blocking the oil passages of small diameter through which the lubricating oil normally flows to the bearings, whereby bearing failures are caused.

The principal objects of the present invention are therefore to provide a lubricating oil composition capable of heavy duty service under varying operating conditions, which compositions shall be effective to reduce or to sub-

2

stantially retard the oxidation of the oil and to inhibit or mitigate the corrosive action of any oxidation or decomposition products which may be formed in the oil.

It is a further principal object of the present invention to provide a lubricating oil composition possessing sufficient reserve alkalinity to neutralize the acid oxidation and decomposition products as they are developed during use of the oil.

It is another principal object of the present invention to provide an anti-oxidant and corrosion-inhibiting lubricating oil composition having detergent or anti-sludge properties.

These objects and others which may appear hereinafter are accomplished by providing compositions suitable for use as improvement agents for hydrocarbon lubricating oils and capable of retarding the deterioration of such oils by oxidation and of neutralizing the acid oxidation and decomposition products which are liberated or formed in the oil during use. In this way, the corrosive and other deleterious effects normally resulting from such acidic products are immediately neutralized and counteracted and conditions detrimental to metallic engine elements are avoided.

This offsetting of the effects of the acid material developed during the use of the oil is accomplished by providing an improvement agent having sufficient latent effective alkalinity or "alkaline reserve" properties capable of acting upon the acid material as it is developed and neutralizing or counteracting the same. This "alkaline reserve" thus represents a latent neutralizing agent which comes into effective operation to neutralize acidic materials when they are liberated.

These improvement agents may be derived from the chemical combination of metallic salts of O,O-diesters of dithiophosphoric acid and ammonia or amines and have the following general structural formula:



wherein each of  $R_1$  and  $R_2$  is an ester-forming member of the group consisting of alkyl, aryl, aralkyl and cycloalkyl radicals;  $Me$  is a metal capable of forming coordination complexes with ammonia;  $z$  is the valence of  $Me$ ; each of  $A$ ,  $B$  and  $C$  is a member of the group consisting of hydrogen, alkyl and alkylol radicals; and  $x$  is an integer from 1 to the coordination number of  $Me$ .

Any O,O-dialiphatic dithiophosphoric acid diester, including the dicycloalkyl dithiophosphoric acid esters, or any O,O-diaryl dithiophosphoric acid diester or any mixed O,O-diester of dithiophosphoric acid may be used in producing the novel products of the present invention. When additive compounds having a relatively high percentage of combined phosphorus and sulfur are desired, as in the production of lubricating oil anti-oxidants having a high activity at relatively low temperatures, it is preferable to employ an O,O-dialkyl dithiophosphoric acid diester in which the alkyl groups are of relatively low molecular weight such as methyl, ethyl, propyl, or butyl radicals. When compounds having a relatively greater solubility in lubricating oils are desired, it is preferable to employ an O,O-dialkyl dithiophosphoric acid diester in which the alkyl groups are of relatively high molecular weight such as those having up to 20 carbon atoms. Such alkyl radicals as lauryl, octadecyl, tetradecyl, etc., may be advantageously used in such a case, since the longer alkyl groups tend to increase the solubility of the dithiophosphates in hydrocarbon lubricating oils. The O,O-diaryl dithiophosphoric acids may frequently be used to advantage as in the production of lubricating oil additives also having a high degree of heat stability wherein

the O,O-diphenyl, O,O-dialkylphenyl, and O,O-dinaphthyl dithiophosphoric acids may be employed. It will be understood that mixed O,O-dithiophosphoric acid diesters may also be employed such as various mixed alkyl-phenyl dithiophosphoric acid diesters.

Any metal may be used in accordance with the principles of the present invention provided it is capable of (1) forming a salt with a dithiophosphoric acid diester, and (2) forming a coordination complex with ammonia or amines. Such metals would include, for example, zinc, copper, chromium, cobalt, nickel and the like. As used herein, therefore, the term "complex-forming" metals will refer to and include such metals. In order to further describe the present invention, the preferred complex-forming metal, zinc, will be used hereinafter primarily for purposes of illustration but it is to be pointed out that such is not to be construed as limitative of the invention and that the other above-mentioned metals may be used.

Ammonia or any suitably reactive amine may be used to form the coordination complex with the zinc, and the term "amine" is understood to include ammonia unless the contrary is indicated. Examples of amines would include ethylamine, propylamine, isopropylamine, ethanolamine, diethanolamine, triethanolamine, cyclohexylamine, cyclopentylamine, di-isopropylamine, diethylamine, guanidine tripropylamine, triethylamine, and the like. The use of an amine containing a long chain hydrocarbon radical is particularly desirable where a greater oil solubility is desired, such as in the use of a lower alkyl diester of dithiophosphoric acid.

With regard to the character "x" as an integer from 1 to the coordination number of the metal used to form the complex salt, it is to be pointed out that its value will depend upon the number of ammonia or amine molecules linked to the zinc salt of the dithiophosphoric acid diester. The maximum value of "x" will therefore be normally twice the valence of the metal and, in the case of zinc, would be 4.

One general method of preparation of the novel products of the present invention comprises the initial formation of the zinc complex with ammonia or an amine, followed by its reaction with the sodium salt of the selected dithiophosphoric diester. For example, a complex-forming metallic salt, such as zinc sulfate (or zinc chloride) may be reacted with aqueous ammonium hydroxide to form zinc ammonium sulfate ( $Zn(NH_3)_4SO_4 \cdot H_2O$ ). This complex salt may then be reacted with the sodium salt of the selected dithiophosphoric acid di-ester to form the zinc ammonium salt of the dithiophosphoric acid di-ester.

Another general method of preparation comprises the initial, separate formation of the zinc salt of the selected dithiophosphoric diester and the direct reaction therewith of the selected amine or ammonia. Such a reaction is exothermic and may be carried out very simply by mixing the reactants together at room temperatures, or at a higher temperature if an accelerated reaction is desired, in the required proportions and permitting the desired reaction to take place. Should it be desired to increase or decrease the temperature of the exothermic reaction mixture, such may be done by appropriate cooling or heating control means, as is well known in the industry.

The invention will be further illustrated in greater detail by the following specific examples. It should be understood, however, that although these examples may describe in particular detail some of the more specific features of the present invention, they are given primarily for the purpose of illustration and the invention in its broader aspects is not to be construed as limited thereto.

#### Example 1

To a solution of 40 grams of sodium hydroxide in 800 ml. of water was added 320 grams dihexylthiophosphoric acid (prepared from methyl isobutyl carbinol). An exothermic reaction started immediately and the temperature of the reaction mixture was held between 25°

and 35° C. The pH of the final solution was adjusted to 10.3 by further addition of sodium hydroxide. 3 grams of "Darco" were added to this solution and, after stirring for 5 minutes, the solution was filtered through a "Hyflo" pre-coated filter to give a clear yellow filtrate. To this filtrate was added a solution of zinc ammonium sulfate prepared by dissolving 143 grams of zinc sulfate and 211 cc. of ammonium hydroxide in about 300 cc. of water. An oily product separated out which was drawn off and stripped under vacuum on a steam bath and filtered through a steam-heated, "Hyflo," pre-coated filter. The final product was a viscous yellow liquid which was soluble in lubricating oil and had the following analysis:

|             | Per cent |
|-------------|----------|
| 15 Nitrogen | 1.86     |
| Phosphorus  | 9.12     |
| Sulfur      | 18.40    |
| Zinc        | 9.56     |

20 This product will slowly crystallize on standing, but this has no effect on its solubility in oil. Warming to 40° or 50° C. will cause the solid material to liquify. The product had excellent detergent properties and possessed considerable "alkaline reserve" and reduced or retarded the 25 deterioration of lubricating oils due to oxidation.

#### Example 2

A solution of sodium dihexylthiophosphate was prepared by adding 160 grams of dihexylthiophosphoric acid (prepared from methyl isobutyl carbinol) to 32 grams of sodium carbonate in 300 ml. of water. The solution had a pH of approximately 8.7 and, after filtering, was treated with a solution prepared by dissolving 72 grams of zinc sulfate heptahydrate and 107 grams 35 ethanolamine in 250 ml. of water. An oily material which separated out was washed with 250 ml. of water and stripped under vacuum on a steam bath to give a viscous liquid material, which was soluble in oil. The product had properties similar to those possessed by the 40 product of Example 1.

#### Example 3

A solution of sodium dihexylthiophosphate was prepared by adding 160 grams of dihexylthiophosphoric acid (prepared from methyl isobutyl carbinol) to 32 45 grams of sodium carbonate in 300 ml. of water. After adjusting the pH to approximately 9.0 by adding 2 grams of additional sodium carbonate, the material was filtered. To the filtrate was added a solution prepared by dissolving 72 grams of zinc sulfate heptahydrate and 124 50 grams of 70% ethylamine in 300 ml. of water. An oily product separated out which was stripped under vacuum on a steam bath and filtered to give a viscous, oil-soluble product having detergent and "alkaline reserve" 55 properties and capable of reducing or retarding the undesirable effects of the oxidation products developed or liberated during use of a lubricating oil.

#### Example 4

To 66 grams of zinc dihexylthiophosphate was added 60 1.7 grams of anhydrous ammonia. An exothermic reaction took place immediately and the temperature of the reaction mixture was held to between 25° and 30° C. The material became quite viscous. After standing several days, the concentrated oil-soluble material crystallized and appeared to be in every way similar to the product resulting from Example 1.

#### Example 5

To 33 grams of zinc dihexylthiophosphate was added 70 10 grams of di-isopropylamine. An exothermic reaction took place immediately and a light yellow viscous oil soluble reaction product resulted. This product was oil-soluble and showed no tendency to crystallize out at any concentration over a period of several weeks and was 75 found to be an excellent lubricating oil additive.

## Example 6

To 33 grams of zinc dihexyldithiophosphate was added 5 grams of triethylamine. A slow exothermic reaction took place and, after warming for some time, to expedite the reaction, a light yellow viscous, oil-soluble reaction product resulted. This product showed no tendency to crystallize out over an extended period of time and was found to be a good improvement agent for lubricating oils and the like.

## Example 7

To 33 grams of zinc dihexyldithiophosphate was added 5 grams of cyclohexylamine. A vigorous exothermic reaction took place immediately resulting in a light yellow viscous, oil-soluble reaction product having the desired detergent, anti-oxidant and corrosion inhibiting properties.

The novel products of the present invention are preferably used in hydrocarbon lubricating mineral oils in relatively small stabilizing amounts which may vary from about 0.1% up to about 4.5% by weight or greater depending on the nature of the particular oil and on the degree of protection desired therein. In automobile engine lubricating oils, stabilizing quantities on the order of from about 0.30% up to about 2.0% by weight are usually incorporated into the oil. Our novel "alkaline reserve" additives, having excellent detergents, anti-oxidant and corrosion inhibiting properties, are compatible with all of the commonly used detergents, stabilizers, sludge inhibitors and other ingredients of compounded oils and may be used in conjunction therewith in smaller or larger quantities, as desired.

If desired, our novel products may be mixed with lubricating oils to form various concentrates, such as for example, a 50% concentrate, and used in such a form rather than in 100% concentrations. Such will facilitate the use thereof and will aid in preventing the crystallization of the product which occurs occasionally with higher concentrations of the ammonia complexes, as noted in Examples 1 and 4.

A representative sample of the product produced as described in Example 1 was tested for efficiency in a Chevrolet L-4 test. This test consists of operating the engine continuously at a speed of 3150 R. P. M. for 36 hours at 30 H. P. loading with a crankcase oil temperature of 280° F. and a water jacket outlet temperature of 200° F. The engine is then disassembled and the parts are inspected and rated. The amount of varnish on the pistons is reported on a scale ranging from 1-10 and 10 means a perfectly clean piston and 1 means a piston which is very dirty with stuck piston rings. The overall rating is reported on a scale ranging from 1-100 in which 100 means a clean engine with no sludge deposits and clean pistons.

The average weight loss per whole bearing may be determined by individually weighing each one of a pair of whole bearings before and after the test with the average of the resulting differences being equal to the average weight loss per whole bearing.

The neutralization number means the alkali equivalent in milligrams of potassium hydroxide which is required to neutralize a gram of the oil.

An S. A. E. 30 Mid-Continent solvent-refined base oil having a viscosity index of 85-95 and with no additive was used as a control and showed the following results:

|                              |         |
|------------------------------|---------|
| Piston rating                | 9.2     |
| Overall rating               | 93.3    |
| Wt. loss per whole bearing   | mgms.   |
| Neutralization number (new)  | 2677    |
| Neutralization number (used) | <0.1    |
| Percent viscosity increase   | 2.7     |
|                              | percent |
|                              | 34      |

0.35% by weight of a zinc ammonium dihexyldithiophosphate was incorporated in a Mid-Continent solvent-

refined base oil similar to the above used oil. The results were as follows:

|                                  |         |
|----------------------------------|---------|
| Piston rating                    | 9.6     |
| Overall rating                   | 97.7    |
| Aver. wt. loss per whole bearing | mgms.   |
| Neutralization number (new)      | 543     |
| Neutralization number (used)     | 0.5     |
| Percent viscosity increase       | percent |
|                                  | 1.4     |
|                                  | 21      |

10 L-1 caterpillar diesel engine test was run on (1) a Mid-Continent solvent-refined base oil containing 0.91% by weight of a detergent commonly used in the industry and 0.79% by weight of a corrosion inhibitor and anti-oxidant also commonly used in the industry and (2) a Mid-Continent solvent-refined base oil wherein a zinc ammonium dihexyldithiophosphate replaced the corrosion inhibitor and anti-oxidant. At the conclusion of the tests, a comparison of the carbon filling in the top ring groove showed an improvement of 30% for the composition containing the ammonium zinc dihexyldithiophosphate.

15 Although we have described but a few specific examples of our invention, we consider the inventive concept not to be limited thereby nor to the specific substances mentioned therein, but to include various other equivalent compounds of similar constitution as set forth in the claims appended hereto. It is understood that any suitable changes or variations may be made without departing from the spirit or scope of the inventive concept.

20 We claim:

30 1. A lubricating oil composition comprising a major portion of hydrocarbon mineral oil subject to oxidation and from about 0.1% to about 5% by weight of a compound having the general formula



35 wherein each of  $R_1$  and  $R_2$  is a member of the group consisting of alkyl, aryl, aralkyl, alkaryl and cycloalkyl radicals;  $Me$  is a metal from the group consisting of zinc, copper, chromium, cobalt and nickel capable of forming coordination complexes with ammonia;  $z$  is the valence of  $Me$ ; each of  $A$ ,  $B$  and  $C$  is a member of the group consisting of hydrogen, alkyl and alkylol radicals; and  $x$  is an integer from 1 to the coordination number of  $Me$ .

40 2. The invention as defined in claim 1 wherein said compound is present in amounts from about 0.30 percent by weight to about 2.0 percent by weight.

45 3. A lubricating oil composition comprising a major portion of a hydrocarbon mineral oil subject to oxidation and from about 0.1% to about 5% by weight of a compound having the general formula



50 55 wherein each of  $R_1$  and  $R_2$  is a member of the group consisting of alkyl, aryl, aralkyl, alkaryl and cycloalkyl radicals; each of  $A$ ,  $B$  and  $C$  is a member of the group consisting of hydrogen, alkyl and alkylol radicals; and  $x$  is an integer from 1 to 4, inclusive.

60 6. A lubricating oil composition comprising a major portion of a hydrocarbon mineral oil subject to oxidation and from about 0.1% to about 5% by weight of a compound having the general formula



65 70 wherein each of  $R_1$  and  $R_2$  is a member of the group consisting of alkyl, aryl, aralkyl, alkaryl and cycloalkyl radicals; and  $x$  is an integer from 1 to 4, inclusive.

75 8. The invention as defined in claim 4 wherein said compound is present in amounts from about 0.30 percent by weight to about 2.0 percent by weight.

6. A lubricating oil composition as defined in claim 1 wherein R<sub>1</sub> and R<sub>2</sub> are alkyl radicals; Me is zinc; x is 2; A, B and C are hydrogen; and x is an integer from 1 to 4, inclusive.

7. A lubricating oil composition as defined in claim 1 wherein R<sub>1</sub> and R<sub>2</sub> are alkyl radicals having six carbon atoms; Me is zinc; z is 2; A, B and C are hydrogen; and x is an integer from 1 to 4, inclusive.

8. A lubricating oil composition as defined in claim 3 wherein R<sub>1</sub> and R<sub>2</sub> are hydrocarbon aliphatic radicals.

9. A lubricating oil composition as defined in claim 4 wherein R<sub>1</sub> and R<sub>2</sub> are hydrocarbon aliphatic radicals.

10. A lubricating oil composition as defined in claim 1

wherein R<sub>1</sub> and R<sub>2</sub> are alkyl radicals; Me is zinc; z is 2; and x is an integer from 1 to 4, inclusive.

11. A lubricating oil composition as defined in claim 1 wherein R<sub>1</sub> and R<sub>2</sub> are alkyl radicals having six carbon atoms; Me is zinc; z is 2; and x is an integer from 1 to 4, inclusive.

References Cited in the file of this patent

UNITED STATES PATENTS

2,344,395 Cook et al. Mar. 14, 1944  
2,382,775 Cook et al. Aug. 14, 1945